

1

2,873,252

## METHOD OF INHIBITING CORROSION OF FERROUS METAL SURFACES

Gustave K. Kohn, Berkeley, Calif., assignor to California Spray-Chemical Corporation, Richmond, Calif., a corporation of Delaware

No Drawing. Application June 24, 1954  
Serial No. 439,158

5 Claims. (Cl. 252—8.55)

This invention relates to an improved method of inhibiting corrosion of ferrous metals and particularly the ferrous metal equipment associated with the production of petroleum hydrocarbons, as in a producing oil well. Additionally, the invention relates to an improved arsenical composition which is adapted for aqueous dilution and suitable for application as a corrosion inhibitor for ferrous metals and particularly as an inhibitor for carbon dioxide-induced metal corrosion.

Ferrous metal corrosion has long been recognized as one of the most serious problems associated with the production and recovery of petroleum hydrocarbons from subsurface formations. The corrosive attack upon the ferrous metal surfaces in contact with the production fluid is primarily due to the action of the weak acidic solutions, such as the aqueous solutions of carbon dioxide, normally present in the production fluid. While the presence of the carbonic acid solutions presumes an acid attack upon the ferrous metal surfaces, other integral and contributing corrosive actions have been recognized. Thus, electrochemical corrosive action is also a major factor.

Although numerous chemical inhibitors have been previously proposed for the treatment of ferrous metal surfaces in contact with corrosive well fluids, it is only recently that any measure of success has been obtained in the practical solution of this problem. It has recently been proposed to inject into the production fluid and circulate throughout the production system an arsenical composition comprising the alkali metal arsenites or alkaline solutions of arsenious oxide. These alkaline arsenical compositions have been used successfully both in the form of dilute aqueous solutions which are pumped or lubricated, intermittently or continuously, into a producing well, or in the form of solid compositions which are dropped into the production tubing and gradually are dissolved into the production fluid. These arsenical corrosion inhibitors provided a tenacious protective film upon the ferrous metal surfaces which successfully inhibits the corrosive action of the contacting production fluid.

In the practical or field application of these alkaline arsenical inhibitors, certain difficulties have been encountered which have prevented the full utilization of the arsenious oxide content of the inhibitor. It has been found that under certain conditions the alkaline arsenicals will form deposits in the form of flocculent precipitates and sludges in the dilution tanks and throughout the injection system associated with the introduction of the inhibitor into a producing oil well.

Basically, in order to achieve a water-soluble, highly-concentrated formulation of arsenious oxide (at least 2 pounds  $As_2O_3$  per gallon), it is necessary to employ a high alkali-arsenic ratio in the formulations. When employing hard waters of at least 70 p. p. m. for dilution in the field mixing tanks, it is noted that deposits are formed throughout the inhibitor system which are largely composed of compounds containing the alkaline earth and heavy metal cations of the dilution water. In extremely hard waters (several hundred p. p. m.), precipita-

2

tion and sludge deposition are almost immediate and voluminous.

Another contributing factor to the formation of deposits on dilution of the alkaline arsenical inhibitors is the presence of antimony impurities associated with the arsenic. Generally, the commercial grades of arsenious oxide contain about 1 to 3 percent of the oxides of antimony and, in the preparation of the alkaline arsenical inhibitors, the conditions of reaction are conducive to the solution of the oxides of antimony with the arsenious oxide. On dilution, irrespective of the hardness of the diluting water, the very low solubility of  $Sb_2O_3$  is approached and the metal surfaces of the tanks, pumps and piping become coated with a sludge high in antimony. 15 A typical analysis of such a coating is as follows:

|                 | Tank Deposit | Valve Deposit |
|-----------------|--------------|---------------|
|                 | Percent      | Percent       |
| $As_2O_3$ ..... | 12.8         | 12.4          |
| $Sb_2O_3$ ..... | 31.6         | 50.8          |

In contrast to the foregoing difficulties in field application of the alkaline arsenical corrosion inhibitors, it has now been found possible to provide a water-miscible arsenical corrosion inhibitor which may be formulated as a concentrate containing at least 2 pounds of  $As_2O_3$  per gallon which is stable in storage; contains negligible quantities of antimony oxides; on dilution with waters having a hardness greater than 70 p. p. m., will not precipitate the alkaline earth and heavy metal cations; and, in general, provides deposit-free operation as a corrosion inhibitor for ferrous metals and particularly the ferrous metal equipment associated with the production of petroleum hydrocarbons.

In accordance with the present invention, it has been discovered that the water-miscible reaction products of arsenious oxide and polyhydric alcohols will provide an arsenical corrosion inhibitor for ferrous metals which possesses materially improved performance characteristics and more universal application over the conventional alkaline arsenical compositions. Although these reaction products result in the formation of arsenite esters, these esters are not necessarily the sole component of the reaction product, which more than likely consists of a mixture of esters and dissolved arsenious oxide.

The properties of the reaction product will vary according to the type of polyhydric alcohol and the mol ratio of reactants employed. The reaction products may vary from a water-miscible, low-viscosity liquid product to a water-miscible, solid or glass-like product. Generally, in order to provide a reaction product possessing optimum water-miscibility and a lower viscosity, it is preferred to react the polyhydric alcohol at such a mol ratio as to provide at least one free hydroxyl group available in the reaction product.

The types of polyhydric alcohols which have been found suitable in the preparation of the arsenical reaction products may be classified into the normally-liquid polyhydroxy aliphatic compounds and the normally-solid polyhydroxy aliphatic compounds. The preferred mol ratios of reactants to produce a stable, water-miscible corrosion inhibitor will lie within the range of 1 mol of arsenious oxide to from 3 to 8 mols of the normally-liquid polyhydric alcohols, and in the range of 1 mol of arsenious oxide to 0.5 to 4 mols of normally-solid polyhydric alcohols.

In the case of the reaction products obtained from the reaction of the normally-solid polyhydric alcohols, as represented by pentaterythritol, the reaction will result in a water-miscible, glass-like reaction product which is emi-

nently suited as a solid arsenical corrosion inhibitor which may be introduced into a producing well in the form of a molded stick and is gradually dissolved in the production fluid to provide corrosion inhibition to the ferrous metal surfaces in contact with the production fluid. An additional advantage of the pentaerythritol arsenical composition is the fact that under certain conditions of operation the solid inhibitor will gradually decompose and release formaldehyde which will afford additional hydrogen sulfide corrosion protection.

Of the normally-liquid polyhydric alcohols, the dihydric alcohols or the glycols containing from 2 to 4 carbon atoms are the most desirable. The glycols, when reacted with arsenious oxide in the mol ratio range of from 3 to 8 mols of glycol per mol of arsenious oxide, will result in a stable, water-miscible, free-flowing product which is readily compounded in concentrations of at least 4 pounds of  $As_2O_3$  per gallon, and may be diluted without deposit formation at the conventional field dilutions of 1 to 30 or greater.

The reaction of the polyhydric alcohols and the arsenious oxide to form the arsenical corrosion inhibitor of the invention inherently avoids the presence of normally-associated antimony in the reaction product. Under the conditions of the reaction, the oxides of antimony do not esterify with the polyhydric alcohols, and the antimony is substantially eliminated in the reaction residue or sludge.

In general, the reaction is conducted by heating the reactants together in the presence of catalytic amounts of a condensing agent, such as about 0.01 to 0.5 percent by weight of a strong mineral acid or a strong base, at a temperature of at least 100° C. and below the boiling point of the polyhydric alcohols. At temperatures approaching 100° C., the reaction is exothermic and proceeds rapidly with the elimination of water. Upon completion of the reaction, the reaction product is immediately applicable as an arsenical corrosion inhibitor.

A number of variations have been employed in carrying out the reaction which may find practical application. Thus, an entraining solvent may be incorporated in the reaction to remove the water formed, and thereby allow a greater control of reaction temperatures. Preparations have been made in the absence of a condensing agent, but such reactions require prolonged heating of the reaction mass in order to complete removal of the reaction water.

The following example is presented as an illustration of the details of the invention.

#### Example

A mixture of reagent-grade arsenious oxide and propylene glycol was incorporated in a reaction vessel in a 6:1 mol ratio of propylene glycol to arsenious oxide. The reaction mass was heated and, as the temperature approached 100° C., catalytic amounts of 50 percent caustic were added. An instantaneous exothermic reaction occurred. The reaction temperature was controlled so that it remained below the boiling point of the propylene glycol. Steam was driven off, and the reaction mass was stirred for 5 to 10 minutes and then cooled. The resulting reaction product was clear, water-white, slightly viscous, but flowable, and water-miscible. When diluted to a 1 to 40 dilution, it did not precipitate either in hard water or when carbon dioxide was bubbled through the solution. When employing technical-grade arsenious oxide containing about 1 to 3 percent of the oxides of antimony, the reaction product is separated from the reaction sludge in which substantially all of the antimony is present.

Additional preparations were conducted employing a

condensing system on the reaction vessel whereby the reaction temperature was controlled to allow the water to escape and refluxing the glycol.

Additional preparations were conducted with ethylene glycol, glycerol, 70 percent commercial sorbitol, 85 percent invert sugar glucose, and pentaerythritol with varying mol ratios to produce stable, water-miscible arsenical corrosion inhibitors which, when evaluated for corrosion inhibition according to the test procedure of Scott and Rohrback published in *Corrosion*, vol. 8, No. 7, pages 234-239, July 1952, showed at least 85 percent corrosion inhibition of ferrous metal surfaces.

Obviously, many modifications and variations of the invention, as hereinbefore set forth, may be made without departing from the spirit and scope thereof, and therefore only such limitations should be imposed as are indicated in the appended claims.

I claim:

1. A method of inhibiting the corrosion of ferrous metals subject to contact with aqueous solutions of carbon dioxide which comprises introducing into contact with said ferrous metals a water-miscible reaction product of  $As_2O_3$  and a polyhydric alcohol obtained at reaction temperatures of at least about 100° C. and below the boiling point of said polyhydric alcohol, said reaction product containing at least one free hydroxyl radical.
2. A method of inhibiting corrosion of ferrous metals which comprises introducing into contact with said ferrous metals a water-miscible reaction product of arsenious oxide and a dihydric alcohol containing from 2 to 4 carbon atoms, said reaction product being obtained by the reaction of 1 mol of arsenious oxide for every 3 to 8 mols of said dihydric alcohol and at reaction temperatures of at least about 100° C. and below the boiling point of said dihydric alcohol.
3. A stable arsenical composition comprising a water-miscible reaction product of arsenious oxide and a normally-solid polyhydric alcohol obtained by the reaction of 1 mol of arsenious oxide to 0.5 to 4 mols of the normally-solid polyhydric alcohol at reaction temperatures of at least 100° C. and below the boiling point of said polyhydric alcohol.
4. A solid arsenical corrosion inhibitor suitable for gradual solution in the production fluid of a producing oil well which comprises a water-miscible reaction product of arsenious oxide and pentaerythritol, said reaction product being obtained by the reaction of 1 mol of arsenious oxide for every 0.5 to 4 mols of pentaerythritol and at reaction temperatures of at least 100° C. and below the boiling point of pentaerythritol.
5. A method of inhibiting the corrosion of ferrous metals which comprises introducing into contact with said ferrous metals a water-miscible reaction product of arsenious oxide and a polyhydric alcohol obtained by the reaction of arsenious oxide with a polyhydric alcohol at reaction temperatures of at least 100° C. and below the boiling point of said polyhydric alcohol and at mol ratios such that said reaction product contains at least one free hydroxyl radical.

#### References Cited in the file of this patent

#### UNITED STATES PATENTS

- |              |                   |               |
|--------------|-------------------|---------------|
| 63,084       | Paraf             | Mar. 19, 1867 |
| 65 1,988,176 | Merrill           | Jan. 15, 1935 |
| 2,346,157    | Farrington et al. | Apr. 11, 1944 |
| 2,635,999    | Rohrback et al.   | Apr. 21, 1953 |

#### FOREIGN PATENTS

- |            |             |               |
|------------|-------------|---------------|
| 70 156,339 | Switzerland | Oct. 1, 1932  |
| 20,665/34  | Australia   | Aug. 21, 1935 |